

## UNITED STATES PATENT OFFICE

2,010,607

PROCESS FOR THE MANUFACTURE OF  
CELLULOSE ESTERSAndreas Ruperti, Basel, Switzerland, assignor to  
the firm of Society of Chemical Industry in  
Basle, Basel, SwitzerlandNo Drawing. Application May 26, 1930, Serial  
No. 455,967. In Switzerland June 1, 1929

5 Claims. (Cl. 8—20)

The present invention relates to the manufacture of cellulose esters and to the products obtained according to the new process.

According to this invention cellulose esters are made by the action of an organic acid anhydride on the group of cellulose derivatives consisting of the cellulose xanthogenates and the cellulose xanthic acid. The esters produced are free from sulfur.

10 The acid anhydride, preferably anhydrides of aliphatic fatty acids, such as the anhydrides of the acetic acid, propionic acid, butyric acid, etc., may be used as such or in a solvent and the reaction may be facilitated by a catalyst. The 15 process is a short one. There are obtained according to the conditions of operation various highly esterified celluloses. Since the operation is conducted in the absence of agents capable of splitting mineral acids and of catalysts having 20 a mineral acid reaction which degrade the cellulose, the cellulose esters formed contain the cellulose in non-degraded form. In esterifying solid cellulose xanthates or cellulose xanthic acid the external form is retained, particularly if the acid 25 anhydride is diluted with a solvent or used in moderate proportion, and if solvents are used which do not dissolve the cellulose xanthogenates and the cellulose esters produced therefrom.

20 The process finds application in many technical operations.

The process is particularly interesting in that it permits of wholly or in part esterifying formed bodies from cellulose xanthates or cellulose xanthic acid, such as threads, bands, films or webs 35 with retention of the external form or the fibrous structure. For example, one may start from threads of a cellulose xanthate or a cellulose xanthic acid made from a viscose solution in the manner usual for making viscose silk but with 40 use of a precipitating bath which, while causing separation of the cellulose xanthate or cellulose xanthic acid wholly or at least in part as such, does not regenerate cellulose, or only in part regenerates it; or it may be from cellulose 45 threads by treatment with alkali and carbon bisulfide, while retaining the fibrous structure and avoiding any dissolving effect during the production. By treating such threads with organic acid anhydride, for instance acetic anhydride, there 50 is obtained a thread which possesses the dyeing properties of a cellulose acetate, being immune towards direct dyestuffs; this is applicable as an effect thread and has considerably enhanced physical properties, particularly in respect of wet and dry tenacity. This tenacity is particularly

pronounced when the operation is conducted in complete absence of conditions which degrade cellulose and in particular when no injurious catalyst has been used. Similarly very valuable are the bodies which may be obtained by impregnating, filling or saturating, dressing or printing the most varied materials, particularly the textile materials, with a solution of viscose, (xanthate), and then treating the material thus prepared with the hot acid anhydride. In this case the cellulose ester is formed in close union with the material and by further treating the latter by a dyeing operation portions of the fibre which have been covered or associated with the cellulose ester are immune to substantive dyestuffs but are dyed by cellulose ester dyestuffs, so that multicolor effects can be obtained. By gentle treatment with acid anhydride the stage of esterification can be kept so low that the new material has the advantage that it is insoluble 10 in most of the commercial solvents of acetate silk. However, by using energetic conditions complete esterification can be obtained. By varying the conditions of operation the lustre of the thread can be retained or affected in any desired manner.

15 The following examples illustrate the invention:—

## Example 1

A cotton web is impregnated with a viscose made in known manner, dried and treated for  $\frac{1}{4}$  to 2 hours with acetic anhydride, if desired in presence of xylene. During this treatment the temperature is raised to 140° C. By this treatment the web acquires a durable dressing stable 30 against water, which gives it a stiff and thick character.

## Example 2

Viscose made by a known process and in a crude or purified condition is locally applied, for instance by printing, to a web or yarn. The material is dried and then treated with hot acetic anhydride, the temperature being, for instance, at the boiling point. The printed places are reserved towards substantive dyestuffs but may be dyed vividly by means of acetate silk dyestuffs, the latter leaving the rest of the material undyed. In this manner various colored effects can be obtained.

## Example 3

A skein of cotton is immersed for 2 hours in an alcoholic potash solution of 20 per cent. strength. Then centrifuged or pressed and for

several hours immersed in carbon bisulfide or subjected to the action of vapor of carbon bisulfide. The skein is gradually converted into cellulose xanthate acquiring a yellow color and 5 becoming soluble in water. After separating the excess of carbon bisulfide the skein is treated with hot acetic anhydride, for instance for 10 minutes to 1 hour at the boiling point of acetic anhydride, or for a longer time at a lower temperature. The 10 fibrous material thus obtained, the composition of which corresponds approximately with a cellulose diacetate, can be dyed vivid and deep tints by means of acetate silk dyestuffs but is completely reserved towards substantive dyestuffs. 15 In chloroform, glacial acetic acid and acetone the fibrous material obtained is insoluble, while in pyridine and nitrobenzene swelling occurs but no dissolution.

*Example 4*

20 Bleached wood pulp is converted in the usual manner into viscose and the latter is spun. As precipitating bath there is used a solution of an alkali salt or an ammonium salt, acidified with acetic acid, or the bath may consist of methyl 25 alcohol mixed with acetic acid. The precipitated thread, soluble in water, is treated with a solution of 20 per cent. strength of acetic anhydride in toluene. The temperature is raised to the boiling point of the solution. There is obtained an 30 ester silk, which has the beautiful lustre, excellent wet tenacity and dyeing properties of acetate silk. In chloroform, acetone, glacial acetic acid, pyridine and nitrobenzene the material obtained 35 is insoluble.

*Example 5*

40 The xanthate thread obtained as described in Example 4 is treated with acetic anhydride at about 100° C., then centrifuged and washed with water. There is thus obtained a lustreless, matte 45 artificial silk. If before the material is washed, the still adhering acetic anhydride is separated by evaporation, the fibre obtained has the usual artificial silk lustre.

*Example 6*

50 A skein of finished cellulose artificial silk (viscose silk, copper silk or nitro-silk) is converted, as described in Example 3, into cellulose xanthate with retention of the fibrous structure and then treated with a solution of 20 per cent. strength 55 of acetic anhydride in xylene for 1 hour at the boiling point. The material increases by about 60 per cent. in weight and has more than double the wet tenacity of the untreated artificial

silk. The dyeing properties of the material are analogous to those of acetate silk; substantive dyestuffs are reserved, acetate silk dyestuffs are absorbed. In acetone, chloroform, glacial acetic acid the material is insoluble.

5 If instead of the solution of acetic anhydride a solution of 20 per cent. strength of maleic anhydride in xylene is used, there is an increase in weight of the material of about 90 per cent. and 10 a yellowish colored product is obtained which is insoluble in chloroform, glacial acetic acid, acetone, pyridine and nitrobenzene, and which has no affinity for substantive dyestuffs.

15 What I claim is:—

1. Process for the manufacture of cellulose esters, characterized by treating that group of cellulose derivatives which consists of the cellulose xanthogenates or of the cellulose xanthic acids with aliphatic carboxylic acid anhydrides in the 20 absence of organic acid halides.

2. Process for the manufacture of threadlike molded articles of cellulose esters which is characterized by treating threadlike molded articles consisting of that group of the cellulose derivatives which consists itself of the cellulose xanthogenates or of the cellulose xanthic acids, with aliphatic carboxylic acid anhydrides in the absence 25 of organic acid halides.

3. Process for the manufacture of bodies of cellulose esters which is characterized by treating products consisting of that group of the cellulose derivatives which consists itself of the cellulose xanthogenates or of the cellulose xanthic acids, with acetic acid anhydride in the absence 30 of organic acid halides.

35 4. Process for the manufacture of cellulose esters characterized by treating that group of the cellulose derivatives which consists of the cellulose xanthogenates or of the cellulose xanthic acids, with aliphatic carboxylic acid anhydrides 40 in the absence of organic acid halides, and in the presence of such diluents which are not capable of dissolving the cellulose esters formed.

45 5. Process for the manufacture of threadlike molded articles of cellulose esters, characterized by treating threadlike molded articles consisting of that group of the cellulose derivatives which consists itself of the cellulose xanthogenates or of the cellulose xanthic acids, with 50 acetic acid anhydride in the absence of organic acid halides, and in the presence of such diluents which are not capable of dissolving the cellulose esters formed.

ANDREAS RUPERTI.